

Jan. 17, 1928.

1,656,892

B. R. SHOVER

METHOD OF MAKING HIGH FINISH SHEETS

Filed April 26, 1922

*Fig. 1.*



*Fig. 2.*



Witnesses:

Edwin Trueb

By:

Inventor:  
BARTON R. SHOVER,  
*R.D. Little*

his Attorney.

Patented Jan. 17, 1928.

1,656,892

UNITED STATES PATENT OFFICE.

**BARTON R. SHOVER, OF PITTSBURGH, PENNSYLVANIA.**

## METHOD OF MAKING HIGH-FINISH SHEETS.

Application filed April 26, 1922. Serial No. 556,740.

This invention relates to ferrous metal sheets and plates having a high finish on one or both surfaces thereof and method of making the same, and has for its principal object 5 the provision of a method that will cheapen the manufacture of such sheets and plates, and produce sheets and plates having a better finish than those produced by any existing methods, of which I am aware, in a rapid 10 and efficient manner.

Heretofore, in the manufacture of high finished ferrous metal sheets or plates for use in making hoods, fenders, and bodies of automobiles, steel furniture and other products requiring a smooth, even finish of paint or enamel, the sheets, after being hot rolled in the usual manner have been pickled or otherwise operated upon to remove the scale and clean them. The cleaned sheets are then annealed and finally are cold rolled to obtain the desired finish. The excessive number of passes through the cold rolls necessary to produce the required finish by cold rolling hardens the sheets to such an extent that they can not be successfully shaped or formed. So the practice heretofore has been to do the major portion of the cold rolling necessary to produce the desired finish, to then again anneal the sheets and then again cold roll them, until the desired finish is obtained, thus necessitating at least two annealing operations and two cold rolling operations to produce the finished sheets. At best, the sheets produced under these conditions are harder and stiffer than desired for a considerable amount of bending or shaping and much harder than if they could be used after annealing and without further cold rolling. However, annealing plates as heretofore made destroys the high finish and they must be again cold rolled to produce such finish.

Many of the finished plates made under existing methods are found to have small surface defects which are not removed by cold rolling, and these plates must then be discarded as seconds or wasters according to the character of the defects.

50 My method consists in the formation on the surface of the sheets, after they are hot rolled, pickled, or otherwise cleaned and, in some cases, annealed, of an alloy which will be softer than the steel of the plates, and then cold rolling the sheets. The cold rolling operation, in addition to reducing the gauge 55 of the sheet, will spread the alloy and fill any

depressions or inequalities in the surfaces of the sheet or plate and results in a smooth surface, with materially less cold rolling than is necessary to finish the ferrous metal sheets as heretofore manufactured. Less pressure extends through the alloy into the ferrous metal sheets, and consequently the sheets are not hardened as much as if they had no alloy applied, and this together with the reduced number of passes necessary to produce the high finish results in high finished sheets that are soft and ductile enough to be readily formed or pressed without a second annealing.

In the drawings, Figure 1 is a sectional elevation showing a sheet having the alloyed surfaces thereon, in readiness for cold rolling.

Figure 2 is a side elevation showing a stand of cold rolls with a sheet or plate therebetween as in the cold rolling operations. 75

In forming the alloy on the ferrous metal sheets or plates 2, after they have been hot rolled and in some cases after they have been annealed, a non-ferrous metal is used, such as zinc or aluminum in coating the sheets or plates, much in the same manner as galvanizing, sherardizing or calorizing is now carried on, so as to provide a non-oxidizing surface on the ferrous metal. This alloy surface on the sheets is formed of a mixture of the ferrous metal of the sheet and the non-ferrous coating metal and consists of an alloy layer 3 integrally united with the ferrous body of the sheet and an extremely thin outer layer 4 of substantially pure coating metal.

It, of course, will be understood that in some cases the alloy surface may be applied to only one side of the ferrous base and also that the alloy coating may be applied or formed on the ferrous base in other ways, such as by hot galvanizing or tinning. 95

After the sheets or plates 2 have the alloy surface formed thereon they are given a number of passes between the cold rolls 5 and 6, which serves to spread the alloy and fill any depressions or inequalities in the surfaces of the sheet and impart a polished high finish to the surfaces. The alloy being softer than the metal of the sheet 2, materially less cold rolling is necessary than would be necessary to finish the materials if they had no alloy surface.

Obviously my improved method can be used in making the materials known to the

trade as strips and cold rolled strips and the terms sheets and plates as used herein are intended to include such strips and cold rolled strips.

5 I claim:—

1. The method of making high finish metal sheets and plates which consists in rolling heated blanks into sheets or plates, preparing the surfaces thereof for coating by pickling the rolled sheets and plates, conditioning the pickled sheets or plates for finishing by coating at least one surface thereof with a softer metal and imparting the high finish to the coated surfaces of the sheets or plates by cold rolling.

2. The method of making high finish metal sheets and plates which consists in rolling heated blanks into sheets or plates, preparing the surfaces thereof for coating by pickling the rolled sheets and plates, conditioning the pickled sheets or plates for finishing by coating at least one surface thereof with an alloy layer of a softer metal and imparting the high finish to the coated surfaces of the sheets or plates by cold rolling.

3. The method of making high finish metal sheets and plates which consists in rolling heated blanks into sheets or plates, preparing the surfaces thereof for coating by pickling the rolled sheets and plates, conditioning the pickled sheets or plates for finishing by coating at least one surface thereof with an alloy layer of zinc and imparting the high finish to the coated surfaces of the sheets or plates by cold rolling.

4. The method of making high finish ferrous metal sheets and plates which consists in rolling heated blanks into sheets or plates, preparing the surfaces thereof for coating by pickling the rolled sheets and plates, conditioning the pickled sheets or plates for finishing by coating at least one surface thereof with a softer non-ferrous metal, and imparting the high finish to the coated surfaces of the sheets or plates by cold rolling.

5. The method of making high finish metal sheets and plates which consists in rolling heated blanks into sheets or plates, softening the rolled sheets or plates by annealing, preparing the surfaces thereof for coating by pickling the annealed sheets and plates, conditioning the pickled sheets or plates for finishing by coating at least one surface thereof with a softer metal, and imparting the

high finish to the coated surfaces of the sheets or plates by cold rolling.

6. The method of making high finish metal sheets and plates which consists in rolling heated blanks into sheets or plates, preparing the surfaces thereof by pickling the rolled sheets and plates, conditioning the pickled sheets or plates for finishing by coating at least one surface thereof with a softer metal, imparting the high finish to the surfaces of the coated sheets or plates by cold rolling and annealing the cold rolled sheets and plates.

7. The method of making high finish metal sheets and plates which consists in rolling heated blanks into multiple length sheets or plates, preparing the surfaces thereof for coating by pickling the rolled sheets and plates, conditioning the pickled sheets or plates for finishing by coating at least one surface thereof with a softer metal and imparting the high finish to the coated surfaces of the sheets or plates by cold rolling.

8. A new article of manufacture consisting of a ferrous metal sheet or plate having the high finish characteristic of cold rolling on at least one surface thereof, said high finish surface being formed of an alloy of the ferrous metal and a softer non-ferrous metal.

9. A new article of manufacture consisting of an annealed ferrous metal sheet or plate having the high finish characteristic of cold rolling on at least one surface thereof, said high finish surface being formed of an alloy of the ferrous metal and a softer non-ferrous metal.

10. A new article of manufacture consisting of a ferrous metal sheet or plate having the high finish characteristic of cold rolling on the surfaces thereof, said high finish surfaces being formed of an alloy of the ferrous metal and a softer non-ferrous metal.

11. A new article of manufacture consisting of a soft annealed ferrous metal sheet or plate having the high finish characteristic of cold rolling on the surfaces thereof, said high finish surfaces being formed of an alloy of the ferrous metal with a softer non-ferrous metal.

In testimony whereof I have hereunto signed my name.

BARTON R. SHOVER.